

# UNITED STATES PATENT OFFICE.

LEE S. CHADWICK, OF EAST CLEVELAND, AND MARC RESEK, OF CLEVELAND HEIGHTS, OHIO, ASSIGNEES TO THE CLEVELAND METAL PRODUCTS COMPANY, OF CLEVELAND, OHIO, A CORPORATION OF OHIO.

## TREATMENT OF IRON OR STEEL FOR THE PREVENTION OF OXIDATION OR RUSTING.

1,388,325.

Specification of Letters Patent. Patented Aug. 23, 1921.

No Drawing.

Application filed October 1, 1917. Serial No. 194,117.

To all whom it may concern:

Be it known that we, (1) LEE S. CHADWICK and (2) MARC RESEK, citizens of the United States, residing at (1) East Cleveland and (2) Cleveland Heights, in the county of Cuyahoga and State of Ohio, have invented a certain new and useful Improvement in the Treatment of Iron or Steel for the Prevention of Oxidation or Rusting, of which the following is a full, clear, and exact description.

This invention relates to improvements in the art of treating iron or steel articles, or articles having a coating of iron or steel, for the purpose of preventing oxidation or rusting thereof, and wherein such articles are provided with a protective covering adapted to render the surfaces thereof capable of resisting, or of being unaffected by, the action of moisture and other oxidizing influences.

It has heretofore been proposed to treat iron or steel or articles composed of or having a surface of iron or steel with a dilute solution of ordinary phosphoric acid ( $H_3PO_4$ ) and preferably in the presence of iron filings or other compound intended to control or regulate the rapidity or strength of the chemical action upon the metal or articles undergoing the treatment.

It has also been proposed to treat such articles by boiling them in solutions of soluble phosphate of iron, manganese or zinc.

The foregoing processes are more or less unsatisfactory for the following reasons:

The coating formed consists essentially of normal or basic phosphates, which are insoluble in water but soluble in even very weak acid solutions. Hence, if any free phosphoric or other acid be present, the coating will dissolve in part at least in such acid, causing the final coating to be thin or uneven and subject to removal, as by rubbing vigorously, especially while wet. If, on the other hand, the solutions employed contain only soluble phosphates of iron, manganese or zinc, without any free acid, the solutions are of themselves so very faintly acid that they will act only on chemically clean iron, free from scale, grease and dirt and, even then, will act only very slowly; hence, articles to be treated in such soluble phosphates require sand-blasting or some similar treatment be-

fore immersion in the solution and then require that they be kept in the solution usually from two to three hours before the treatment is completed.

By our method of treatment, we are enabled to produce a rust-proof coating on iron or steel parts in which the coating can be obtained in a much shorter time than is required by any previous process, with less preliminary treatment of the metal and at a material saving of expense; furthermore, the resultant coating is denser, harder, and more uniform, and hence superior in its rust-resisting qualities to the coatings produced by any of the previously proposed processes with which we are familiar.

It is well known that if iron is immersed in certain metallic salts, the iron will be dissolved and the metal of that salt deposited. This is because the metal in the salt is less basic than iron; that is, less electro positive; hence iron tends to replace it in the solution to form a more stable compound with the acid radical than the other metal did. The speed with which this action goes on, however, depends on the relative strength of the acid radical and the basic radical, the change being rather rapid in solutions having an acid reaction and proceeding more slowly in nearly neutral solutions.

The common metals which iron will replace in this manner in the solutions of their salts are lead, bismuth, tin, copper, mercury, silver and gold. Now the di-hydrogen phosphates of most of these metals are soluble and have an acid reaction when dissolved in water. Hence, if iron or steel articles are placed in solutions containing soluble di-hydrogen phosphates of any of these metals, two reactions go on simultaneously. In one, iron replaces the metal in the phosphate. In the other, iron combines with the soluble di-hydrogen phosphate to form an insoluble normal phosphate. When the work is first placed in the bath, the first reaction predominates; but, as the phosphate coating grows heavier, or builds up, less of the metal is deposited. The final coating consists of a mixture, or compound, of normal phosphates of iron and of the metal in the salt, together with some of the metal itself deposited in with the phosphates. While other reactions may proceed to a slight extent between the

metals and the phosphates, they do not progress to an extent to affect the resultant coating.

- As the action of the salt in dissolving the iron proceeds rather rapidly when the work is first placed in the bath, the work is cleaned of scale or dirt and of thin films of oil within the first few minutes following the insertion of the work in the bath, which results in a very uniform coating being produced in a very short time and without preliminary treatment. In case the work contains much grease, the only treatment needed is to wash it in naphtha, or some similar solvent.
- It will be noted that this action is entirely different from any that can take place with salts of any of the metals previously used for rust proof work, for these metals are not less electro-positive than iron and, consequently, they will not be deposited along with the phosphates.

While this process may be carried out by the use of any soluble phosphate of the metals less basic than iron, in practice we ordinarily employ mixtures of copper di-hydrogen phosphate and copper mono-hydrogen phosphate, the presence of the mono-hydrogen phosphate insuring the absence of all free acid. These copper phosphates may be made in a number of different ways, as, for instance:

30 pounds of blue vitriol or copper sulfate crystals are dissolved in ten gallons of boiling water. Phosphate of soda is dissolved in hot water and added to the foregoing solution in such proportion as to turn red litmus paper slightly blue; this usually requires from 50 to 90 pounds of phosphate of soda, depending on its strength. Then take about one-half as much phosphate of soda as has been used before, place in a copper can and add to it about 14 pounds of sulfuric acid testing 66° Baumé, adding enough water to cause the phosphate to dissolve in the acid. Then add the second solution to the first solution in a mixing tank and add enough water to make a total of about 60 gallons, stirring very thoroughly. The phosphate of soda referred to above is di-sodium mono-hydrogen phosphate  $Na_2HPO_4$ . As the amount of moisture contained in the phosphate of soda varies, the amount to be used must be judged by its chemical effect and this amount will vary from time to time for reasons stated.

The products formed are copper di-hydrogen phosphate, copper mono-hydrogen phosphate, and sodium sulfate. As the sodium sulfate formed is inert, it is not necessary to remove it from the solution. By varying these proportions the various quantities of di-hydrogen and mono-hydrogen phosphates present can be changed as desired.

65 The work to be treated is hung in a tank

containing 500 gallons of water to which 3 or 4 gallons of the mixture, produced as heretofore described, has been added, and the contents of the tank are heated to the boiling point. For every batch of additional work, about 1 gallon of the mixture will be added. After boiling in this solution for a period of from thirty minutes to an hour, the parts are, under ordinary conditions, completely and satisfactorily coated. The 70 coating produced is of a dull copper color, hard, dense and uniform and contains a sufficient quantity of metallic copper so that it may be plated. After being taken from the bath, the parts may be oiled or otherwise 80 treated as desired.

Instead of using a phosphate or phosphates of copper, we may use the soluble phosphates of one or more metals one of which at least should be less basic than iron. 85

Still another method is to add to bone ash—consisting principally of  $Ca_3(PO_4)_2$ —two-thirds of its weight of sulfuric acid and two-thirds of its weight of blue vitriol. This will precipitate calcium sulfate and leave in solution copper-di-hydrogen phosphate, which can be drawn off. Sodium phosphate may then be added to the solution until the desired quantity of mono-hydrogen phosphate is formed. 95

A further and important advantage of our process is that it enables us to employ a relatively cheap acid (sulfuric acid), thereby cheapening the cost of the rust-proofing operation. Furthermore, as pointed out hereinbefore, this low cost of ingredients is attended with a shorter period of treatment and with the production of a coating superior to that secured by the practice of any other process with which we are familiar. 100 In our patent #1,320,734, we have described compounds and a process for coating metal wherein the ingredients of the compounds include an alkali phosphate, copper sulfate, and sulfuric acid, and wherein certain features disclosed therein are covered broadly by the claims. In this application, we disclose compounds which have the advantage, over those disclosed in said patent, of producing both the di-hydrogen phosphate 110 and the mono-hydrogen phosphate of metals less basic than iron, also the use of soluble phosphates of a plurality of metals, at least one of which is less basic than iron. 115

Having thus described our invention, what we claim is:—

1. The process of treating iron or steel, or articles composed of or having a surface of iron or steel, which includes subjecting the said articles to the action of a bath containing a mixture of di-hydrogen and mono-hydrogen phosphates of a metal less basic than iron. 125

2. The process of treating iron or steel, or articles composed of or having a surface of 130

iron or steel, which includes subjecting the said articles to the action of a bath containing a mixture of copper di-hydrogen phosphate and copper mono-hydrogen phosphate.

5. A compound for treating iron or steel containing mixtures of di-hydrogen and mono-hydrogen phosphates of a metal less basic than iron.

10. A compound for treating iron or steel containing a mixture of copper di-hydrogen phosphate and copper mono-hydrogen phosphate.

15. The process of treating iron or steel, or articles composed of or having a surface of iron or steel, which includes subjecting the said articles to the action of a bath containing phosphates of a metal less basic than iron.

6. The process of treating iron or steel or

articles composed of or having a surface of 20 iron or steel which includes subjecting the said articles to the action of a bath containing a mixture of metallic phosphates at least one of which phosphates is of a metal less basic than iron.

25. 7. The process of treating iron or steel or articles composed of or having a surface of iron or steel which includes subjecting the said articles to the action of a bath containing a metallic di-hydrogen phosphate and a 30 metallic mono-hydrogen phosphate, the di-hydrogen phosphate being of a metal less basic than iron.

In testimony whereof we hereunto affix our signatures.

LEE S. CHADWICK.  
MARC RESEK.